

# United States Patent [19]

Johansson

[11] 3,912,836  
[45] Oct. 14, 1975

[54] PROCEDURE FOR SURFACE TREATMENT OF WOOD

[75] Inventor: Karl Ingvar Georg Johansson, Spanga, Sweden

[73] Assignee: Erik Gustav Lennart Eriksson, Valberg, Sweden

[22] Filed: Apr. 25, 1973

[21] Appl. No.: 354,446

## Related U.S. Application Data

[63] Continuation-in-part of Ser. No. 351,161, April 16, 1973, abandoned.

## Foreign Application Priority Data

Apr. 27, 1972 Sweden..... 5623/72

[52] U.S. Cl..... 427/341; 427/342

[51] Int. Cl.<sup>2</sup>..... B05D 3/04; B05D 3/10

[58] Field of Search..... 117/148, 62; 427/317, 325, 427/341, 342, 393, 397, 440

## References Cited

### UNITED STATES PATENTS

|           |         |                   |         |
|-----------|---------|-------------------|---------|
| 2,114,784 | 4/1938  | Maisch.....       | 117/57  |
| 2,140,981 | 12/1938 | Booty et al. .... | 117/59  |
| 2,174,132 | 9/1939  | Maisch.....       | 117/148 |
| 2,330,826 | 10/1943 | Hunn .....        | 117/148 |
| 2,350,135 | 5/1944  | Stamm .....       | 117/148 |
| 2,352,740 | 7/1944  | Shannon .....     | 117/59  |
| 2,363,658 | 11/1944 | Decker .....      | 117/148 |
| 2,572,070 | 10/1951 | Stamm et al. .... | 117/57  |

|           |         |                       |         |
|-----------|---------|-----------------------|---------|
| 2,674,543 | 4/1954  | Iablokoff.....        | 117/59  |
| 2,740,728 | 4/1956  | Sonnabend et al. .... | 117/59  |
| 2,947,648 | 8/1960  | Sonnabend et al. .... | 117/59  |
| 3,219,473 | 11/1965 | Dimond .....          | 117/148 |
| 3,476,585 | 11/1969 | Fraser .....          | 117/57  |
| 3,547,679 | 12/1970 | Moran .....           | 117/59  |
| 3,636,199 | 1/1972  | Jenks et al. ....     | 117/148 |

Primary Examiner—Michael Sofocleous

## ABSTRACT

A wood treatment involving pretreatment of the wood surface with an agent facilitating penetration of impregnant into said surface, a pretreatment agent being chosen in the form of a condensable or polymerisable, hydrophilic substance in liquid form, which is free from solvent and causes the wood to swell or dissolves its constituents, with which substance the wood surface is pretreated and impregnated, to a depth of a few millimetres, after which the substance is caused to harden either by subsequent treatment with hardeners and heat treatment or by corresponding subsequent treatment with an agent which can be caused to react with the pretreatment agent under formation of a polymer. The pretreatment takes place with a solution of formaldehyde and/or low molecular paraformaldehyde in phenol or substituted phenol, and the so pretreated wood is treated with acid or alkaline vapours for starting of hardening, and further a heat treatment is added which may be combined with a mechanical treatment of the wood surface.

5 Claims, No Drawings

## PROCEDURE FOR SURFACE TREATMENT OF WOOD

The present application is a continuation-in-part of my earlier application Ser. Number 351,161 filed Apr. 16, 1973 now abandoned.

The French Patent No. 2,113,481 relates to a procedure for surface treatment of wood, the surface layer of the wood being pretreated with an agent which facilitates penetration of impregnant into the wood surface. Characteristic of said patent is that as pretreatment agent is used a condensable or polymerizable, hydrophilic substance in liquid form, free from solvent, causing the wood to swell or dissolving wood constituents, with which substance the wood surface is pretreated and impregnated, preferentially to a depth of at most a few millimetres but even up to one-fifth of the thickness of the wood, after which the substance is caused to harden either by subsequent treatment with hardeners and heat treatment or by corresponding subsequent treatment with an agent which can be caused to react with the pretreatment agent under formation of a polymer.

The object of the present invention is to further develop said surface treatment procedure and to indicate treatment agents usable for industrial application.

The invention is characterized in that the pretreatment is done with a solution of formaldehyde and/or low molecular paraformaldehyde in phenol and/or substituted phenol, and in that the so pretreated wood is treated with acid or alkaline vapours for starting of the hardening reaction, and that an, in itself, known heat treatment takes place, which may be combined with a likewise known mechanical treatment of the wood surface.

According to one embodiment the pretreatment is done at elevated temperature, after which the hardening is done by subsequent treatment with ammonia in gaseous form and heating.

Alternatively the pretreatment can be done at room temperature and to the pretreatment agent is added an ammonium salt of a strong acid, e.g. ammonium chloride or some other salt, e.g.  $\text{AlCl}_3$ , which at room temperature does not appreciably affect the pretreatment agent but in the subsequent treatment is decomposed by heat and gives off gases, so that hardening of the pretreatment agent occurs.

The pretreatment can be done at atmospheric pressure or a slight overpressure, the pretreatment agent being caused to penetrate preferentially into cell walls and cavities in the surface layer of the wood. Alternatively the pretreatment can be done at elevated pressure, the pretreatment agent being caused to penetrate more deeply, after which the hardening is done at elevated temperature.

The invention will now be explained in greater detail with reference to some embodiments.

### EXAMPLE 1

Boards of pinewood are impregnated with a solution of formaldehyde in phenol in the proportion (weight) 1:1.8 obtained either through coalescence of paraformaldehyde and phenol or through absorption of gaseous formaldehyde in molten phenol at 60°-100°C and at an overpressure of 1-5 kp/cm<sup>2</sup> during 30-60 min. The impregnation solution is tapped off and the impregnation container is filled with ammonia gas to an overpressure

of 0.5-2 kp/cm<sup>2</sup> during 30-60 min, after which the wood material is heated to 80°-100°C for 1-4 hours. If a glossy surface of the material is desired, a hot pressing operation can finally be done, e.g. at an overpressure of 2-10 kp/cm<sup>2</sup> and 140°C for 1-10 min. The boards so treated, which, dependent on the thickness of the wood, contain 10-20 % plastic concentrated at the surface layer of the wood, have a very satisfactory hardness and abrasion resistance and can suitably be used as floor material.

### EXAMPLE 2

Boards of spruce are impregnated with a solution of 1 part by weight formaldehyde in 1.8 parts by weight 15 of a mixture of phenol and a halogenized phenol, e.g. p-chlorophenol, at 60°-100°C. For this purpose the boards are placed in a pressure cylinder of conventional type and subjected to a slight overpressure of 1-4 kp/cm<sup>2</sup>. The pre-treatment solution is then pumped 20 into the cylinder and the pressure is raised to 10-15 kp/cm<sup>2</sup>, so that a quicker and deeper penetration of the wood material is obtained. After 0.5-3 hours the remaining pretreatment agent is tapped out of the cylinder and, owing to the pressure applied in advance, the 25 solution which has not penetrated into the cell walls is now pressed out of the wood, so obtaining an impregnation primarily of the cell walls. Thereafter the impregnation container is filled with ammonia gas to an overpressure of 0.5-2 kp/cm<sup>2</sup> for 30-60 min. and the 30 material is then heated to 80°-100°C for 1-4 hours. This produces a wood material containing 10-30 % plastic with very good strength properties, an excellent dimensional stability and good fire resistance, which is suited for use under severe conditions out-of-doors.

### EXAMPLE 3

Pieces of plywood are immersed in a solution of formaldehyde in phenol in the proportion 1:1.8, in which is dissolved 0.5-5 % ammonium chloride. The 40 pieces of wood are left to absorb the solution during 15-60 min. and are then taken up and heated in a heating furnace at 80°-100°C for 1-2 hours. The resulting product has a good abrasion resistance and ability to 45 resist both water and alkali.

### EXAMPLE 4

The surface chips for chipboards are sprayed with a solution of formaldehyde in phenol in the proportion 1:1.8 in which 0.5-5 % ammonium formate has been 50 dissolved. The weight of added solution is 10-50 % of the weight of the surface chips. The spreading and compression of the surface chips are done in the conventional way at, for example 150°C, 20 kp/cm<sup>2</sup> and 5 min, and the resulting chipboard has considerably 55 improved surface density properties.

### EXAMPLE 5

Veneer is treated on both sides with a solution of formaldehyde in phenol as in the preceding example, is 60 hardened and used as surface layer, possibly also intermediate layer, for the manufacture of plywood, which thereby acquires good abrasion resistance, excellent adhesion between the layers and good water repelling properties.

### EXAMPLE 6

Telegraph poles, fencing poles, railway sleepers or

similar heavy timber, are impregnated with a solution of formaldehyde in phenol in the proportion 1:1.8 for 1-2 hours at 60°-100°C and at an overpressure of 2-10 kp/cm<sup>2</sup>. Thereafter the impregnation solution is tapped off and the impregnation tank is filled with NH<sub>3</sub> gas to an overpressure of 1-5 kp/cm<sup>2</sup> at a temperature of 80°-100°C for 1-2 hours. The wood material so treated contains 5-15% plastic to a depth of 5-15 mm, which gives it an excellent surface hardness, a good rotproofness and an improved flexural strength. The thickness of the treated surface layer permits, for example, the use of climbers on telegraph poles treated in this way without breaking through the resulting surface layer.

## EXAMPLE 7

Dried plywood veneer is immersed in a solution of formaldehyde in phenol in the proportion 1:1.8 for 1-10 min at 0-2 kp/cm<sup>2</sup> overpressure. The sheets of veneer are prehardened in a heating furnace at 50°-100°C in an ammonia gas atmosphere for 15-60 min and are thereafter used in the conventional way as face veneer in plywood manufacture. The resulting plywood product has an excellent surface hardness and abrasion resistance and good resistance to moisture and alkali.

What is claimed is:

1. A process for the surface-treatment of wood, which comprises pretreating a wood substrate at a temperature between about 60°-100°C. for about 1 to 2 hours with a hydrophilic liquid material, that is substantially free of any solvent and that causes the wood to swell or dissolves constituents of the wood, until the desired depth of penetration has been attained; said hy-

drophilic liquid material consisting of a condensable solution of formaldehyde in phenol in the weight ratio of about 1:1.8; and thereafter at a temperature between about 50° and about 150°C. treating the resulting pretreated wood with a condensing agent for a time sufficient to obtain a hardened condensate of said hydrophilic material in the form of an abrasion resistant surface.

2. A process according to claim 1, in which the treating agent is gaseous ammonia.

3. A process according to claim 1, in which the formaldehyde is present as paraformaldehyde.

4. A process for the surface-treatment of wood, which comprises pretreating a wood substrate at room temperature with a hydrophilic liquid material, that is substantially free of any solvent and that causes the wood to swell or dissolves constituents of the wood, until the desired depth of penetration has been attained; said hydrophilic liquid material consisting of a condensable solution of formaldehyde and a heat-decomposable ammonium salt in phenol in which the weight ratio of formaldehyde to phenol is about 1:1.8; and thereafter heating the pretreated wood at a temperature of about 80° to about 150°C for a time sufficient to decompose the ammonium salt to ammonia and to obtain a hardened condensate of said hydrophilic material in the form of an abrasion resistant surface.

5. A process according to claim 4, in which the heat-decomposable ammonium salt comprises ammonium chloride.

\* \* \* \* \*

35

40

45

50

55

60

65